

## UNITED STATES PATENT OFFICE

2,360,283

## COBALT SICCATIVES

John T. Rutherford, Berkeley, Calif., assignor to  
Standard Oil Company of California, San Fran-  
cisco, Calif., a corporation of Delaware

No Drawing. Application August 27, 1938,  
Serial No. 227,178

5 Claims. (Cl. 260—439)

This invention relates to methods of preventing the deterioration of cobalt siccatives and to cobalt siccatives rendered permanently oil-soluble and resistant to color change. It has particular reference to a stabilized cobalt naphthenate siccative for employment in paints, varnishes, ink oils and the like as a drying agent.

Prior to its incorporation in paints, varnishes and the like, cobalt naphthenate is often dispensed and stored as an essentially pure dry solid, sometimes in massive and sometimes in finely pulverized form. Upon storage, and particularly upon exposure to air, cobalt naphthenate deteriorates to such an extent that considerable proportions become insoluble in oil, whether by the formation of oxides or of oil-insoluble salts is not exactly understood. This degradation of cobalt naphthenate, which in its normal state is completely oil-soluble, is manifested by a progressive change in color, from an original deep blue-purple to a green and finally to a brown. As these color changes take place, the naphthenate becomes progressively less soluble in petroleum thinners and drying oils, rendering it useless as a paint drier; for example, a finely pulverized cobalt naphthenate may become entirely insoluble in oil and thinners upon the lapse of some months, when exposed to the air.

Likewise prior to its incorporation in paints, varnishes and the like, cobalt naphthenate is often manufactured, dispensed and stored in solution in petroleum thinners and drying oils, usually in quite concentrated solutions. The surface films of such solutions, for example container walls occasionally splashed by the liquid but normally above liquid level, also suffer the above deterioration in oil-solubility to a greater or less extent, which deterioration is likewise accompanied by the color changes referred to.

It will be understood that these deteriorations in the cobalt naphthenate itself are of but little if any consequence in the event that they are initiated only subsequent to the final incorporation of the drier in the paint or varnish in which it plays its part as a drying accelerator, as such deterioration is masked or perhaps prevented by the preponderant amounts of vehicles, pigment, etc. with which it is then associated. It will accordingly be understood that the effects described, and the invention here disclosed, are concerned entirely with the drier itself, in solid or in dissolved or so-called "liquid" form, before incorporation in the preponderant amounts of vehicles and pigments which together con-

stitute an ultimate paint, varnish, ink oil or the like type of composition.

It has now been found that the intimate admixture of a very small amount of certain inhibiting agents will remarkably postpone the above deterioration or degradation, that in the presence of such agents the cobalt naphthenate retains its original complete solubility in thinners and oils, and that the color changes which normally accompany the usual progressive deterioration do not manifest themselves with their normal rapidity. In general, the agents found to stabilize cobalt naphthenate against the untoward degrading effects here noticed are the aromatic hydroxy compounds, and derivatives of aromatic-hydroxy compounds, as more fully exemplified herein below.

It is a purpose of this invention to disclose and provide cobalt naphthenate compositions, as solids and as solutions in oils and thinners, which do not deteriorate to form oil-insoluble substances at the normal rates at which such deterioration occurs, and to disclose and provide methods by which such stabilization may be accomplished. It is a further object of this invention to disclose and provide cobalt naphthenate compositions, in dissolved as well as in undissolved form, which contain aromatic-hydroxy compounds in sufficient amount and in sufficient intimacy of association to effect these stabilizations against color- and solubility-alterations.

In exemplification of the methods and compositions of the invention:

Inasmuch as the initiation and progress of oil-insolubility of cobalt naphthenate have been found to be manifested through accompanying changes in color, it has been found convenient to measure the effectiveness of the inhibiting agents by the observation of such color changes, for example in the following manner: Ordinary analytical filter paper is dipped in a solution of the cobalt naphthenate in a volatile mineral thinner, or some drops of such a solution are allowed to fall upon such a porous paper. The thinner rapidly evaporates, leaving a residue of very finely divided solid cobalt naphthenate of extensive surface area. The paper is exposed to the air and is observed periodically for such color changes as may appear in the solid cobalt naphthenate particles, such color changes taking the following course: purple (original), greenish traces, green, dark green, brown (ultimate). Ordinarily the progress toward dark green is sufficient to ascertain the effectiveness of the

substances under test for inhibitory power. The inhibiting agents themselves are dissolved or dispersed in the volatile mineral thinner employed as the solvent in the conduct of such tests, thus providing for intimate admixture with the cobalt naphthenate upon evaporation of the solvent.

The tabulation shows the manner in which small amounts of various of the aromatic-hydroxy compounds operate for the prevention of oil-insolubility, as indicated by progressive color changes observed in the manner described.

|                                                          | Number of days before first appearance of— |       |            |
|----------------------------------------------------------|--------------------------------------------|-------|------------|
|                                                          | Greenish traces                            | Green | Dark green |
| Cobalt naphthenate alone.....                            |                                            |       |            |
| +1.0% pyrogallol.....                                    | >20                                        | 7     | 11         |
| +0.1% 240-300° C. wood tar distillate cresols.....       | >20                                        | >20   | >20        |
| +1.0% 180-205° C. cracked petroleum naphtha cresols..... | 13                                         | 13    | >20        |

Generally, from 0.05% to 2.0% by weight of the aromatic-hydroxy compounds, based on the cobalt naphthenate and intimately admixed with it in either solid or dissolved form, will be found sufficient for the purposes of the invention. Amounts of these compounds as high as 5% by weight will in most cases cause only an inconsiderable improvement over the employment of 2.0% by weight.

The mono-, di-, tri- and poly-phenols and their alkyl derivatives, such as the methyl, ethyl, propyl, isopropyl, butyl, isobutyl and higher homologues, the cresols, hydroquinone, phloroglucinol, pyrocatechol, pyrogallol, resorcinol and the naphthols, especially beta-naphthol, as well as the acyl derivatives thereof, such as the acetyl, propionyl, butyryl, valeryl and higher homologues thereof, may be employed in the practice of the invention.

In preparing the compositions of the invention, intimate admixture of the stabilizing agent with the cobalt naphthenate is essential. This may be accomplished by dissolving the requisite amount of the agent in a solvent and dispersing it on the surface of the solid particles of cobalt naphthenate; the evaporation of the solvent leaves a residual quantity of the agent in sufficiently widely dispersed form. In the event that the cobalt naphthenate is manufactured in "liquid" form, that is, in solution in a thinner or solvent, the agent may merely be incorporated in the solvent itself; or the inhibitory substance may be added during the course of the formation of the metal naphthenate salt itself, so long as the progress of the formation allows it to accompany the naph-

thenate and remain permanently and intimately associated therewith. The principal desideratum here is that the aromatic hydroxy compound may be allowed to function in the manner intended

5 for the practice of the invention, namely, in sufficient amount and in sufficiently intimate association with the cobalt naphthenate to enable it to inhibit or entirely prevent the deteriorations in oil-solubility and color referred to herein above.

10 Certain obvious modifications of the invention as above described will be apparent to one skilled in the art, and it will be understood that while the character of the invention and numerous 15 illustrative examples of its practice have been described in detail, this has been done by way of illustration only and with the intention that no limitation be imposed upon the invention, which includes all such changes and modifications as come within the scope of the appended 20 claims.

I claim:

1. A cobalt naphthenate siccative stabilized against color change and decrease in oil solubility comprising cobalt naphthenate and an inhibiting agent comprising a cresol, said cobalt naphthenate without said inhibiting agent being subject to color change and decrease in oil solubility, and said inhibiting agent being mixed with said cobalt naphthenate in a proportion 30 sufficient to inhibit color change and decrease in oil solubility of said cobalt naphthenate.

2. A cobalt naphthenate siccative stabilized against color change and decrease in oil solubility comprising cobalt naphthenate and an inhibiting agent comprising 180-205° C. cracked petroleum naphtha cresols, said cobalt naphthenate without said inhibiting agent being subject to color change and decrease in oil solubility, and said inhibiting agent being intimately mixed 40 with said cobalt naphthenate in a proportion sufficient to inhibit color change and decrease in oil solubility thereof.

3. A cobalt naphthenate siccative stabilized against color change and decrease in oil solubility comprising cobalt naphthenate and between 45 0.05% and 5.0% of its weight of a cresol.

4. A cobalt naphthenate siccative stabilized against color change and decrease in oil solubility comprising cobalt naphthenate and between 50 0.05% and 5.0% of its weight of cracked petroleum naphtha cresols.

5. A cobalt naphthenate siccative stabilized against color change and decrease in oil solubility comprising cobalt naphthenate and between 55 0.05% and 5.0% of its weight of a 180-205° C. fraction from cracked petroleum naphtha cresols.

JOHN T. RUTHERFORD.